

M. J. WALSH,  
METHOD OF CASTING STRAP BACK BRAKE SHOES,  
APPLICATION FILED NOV. 9, 1917.

1,315,804.

Patented Sept. 9, 1919.



FIG. 1

FIG. 2



FIG. 3

Inventor  
Michael J. Walsh  
By  
*J. J. Walsh & Sons Co.*  
Attys.

# UNITED STATES PATENT OFFICE.

MICHAEL J. WALSH, OF MONTREAL, QUEBEC, CANADA.

## METHOD OF CASTING STRAP-BACK BRAKE-SHOES.

**1,315,804.**

Specification of Letters Patent. **Patented Sept. 9, 1919.**

Application filed November 9, 1917. Serial No. 291,159.

*To all whom it may concern:*

Be it known that I, MICHAEL J. WALSH, a subject of the King of Great Britain, and resident of the city of Montreal, in the Province of Quebec and Dominion of Canada, have invented certain new and useful Improvements in Methods of Casting Strap-Back Brake-Shoes, of which the following is a full, clear, and exact description.

10 This invention relates to improvements in method of casting brakeshoes and other articles, and more especially to a method of casting articles in which some member is located in the mold, so as to be incorporated 15 in the casting. This method will, therefore, apply particularly to the casting of strap back brakeshoes.

The object of the invention is to provide a simple and expeditious method of casting 20 articles in metal, which will yield a high grade of output.

A further object is to provide a method of securing inserts in the mold, so that they may be incorporated in the castings.

25 It has been customary in the past to cast articles such as brakeshoes on end, but it has been found that this method is liable to produce poor castings. Articles which are required in large numbers with smooth sur-

30 faces are frequently cast in metal molds. These molds are in themselves rigid, and also have a certain definite expansion and contraction which must be taken into consideration, as well as the expansion and con-

35 traction of the metal poured into them. When articles such as brakeshoes are cast on end, the cope and drag of the mold are usually tightly secured together to prevent the formation of fins on the casting at the part-

40 ing line of the molds. This does not permit of any relative movement of the mold parts with the expansion and contraction of either themselves or the metal poured into them. Attempts have been made to overcome this

45 by pressing one of the parts against the other by means of springs or elastic fluid such as air, but the results produced by such methods are not entirely satisfactory. Springs lose their temper and power when they become

50 heated, and the other appliances are cumbersome, complicated and expensive. It has also been proposed to make molds which are expandible and contractible in all directions, in order to accommodate the mold to the ex- 55 pansion and contraction of the metal poured into it.

According to this invention, a mold is produced having the ability to expand in one or two directions, or possibly in both directions simultaneously. The mold is the 60 subject matter of application 201,160, filed Nov. 9, 1917. In casting elongated articles, it is obvious that most of the expansion will be in the longitudinal direction and that any tendency to expansion in other directions 65 will readily convert itself to expansion in the longitudinal direction, if the mold is rigid in the transverse direction but free to expand longitudinally. The mold is disposed in an inclined position, so that the 70 cope is supported on the drag and presses down on the same by the action of gravity. The cope forms one end of the mold and the drag forms the opposite end, so that when the metal poured into the mold expands, the cope may slide slightly on the drag and yield to the expansion, thus over- 75 coming the necessity for expansibility in other directions, and preventing the cope from being lifted off the drag by the ex- 80 pansion of metal or the metal being forced into the parting line so that fins are pro- 85 duced on the casting. The drag is support- 90 ed in an inclined position, the inclination being such that the metal will run freely to the lower end of the mold, and also such that the cope will rest solidly on the drag. In order to enable the expeditious carrying 95 out of the method, the molds may be ar- ranged in batteries, the drags being suitably supported and the copes being provided with means for quickly lifting them to re- 100 move the casting and permit the mold to cool.

In casting strap back brakeshoes, great 95 difficulty has been experienced in supporting the strap back in the mold, so that it presses tightly against the mold and prevents the entrance of molten iron between it and the mold. Difficulty has also been experienced 100 in accurately positioning the strap back in the mold. These difficulties are peculiar to casting brakeshoes on end.

The present improved method enables the strap backs to be secured firmly in the cope, 105 so that the tendency of the molten iron to force its way between the strap back and the cope is reduced to a minimum. The position in which the brakeshoe is cast enables external means to be used for supporting 110 the strap back in the mold, so that all internal supports may be dispensed with. The

inclined casting position also reduces to a minimum the possibility of molten iron escaping through the mold opening necessary for the external support of the strap back.

5 In the drawings the invention is illustrated as applied to the casting of strap back brakeshoes, but it will be understood that it is not limited to this particular branch of the art, as it may be applied to other articles.

10 In the drawings:—

15 Figure 1 is a sectional view of a brakeshoe mold.

Fig. 2 is an end elevation thereof.

20 Fig. 3 is a section on the line 3—3, Fig. 1.

25 Referring more particularly to the drawings, 11 designates the drag and 12 the cope of a brakeshoe mold. The drag is provided with an end member 13 overlapping the end of the 30 cope, and provided with a groove or runner 14 through which the molten metal is led into the mold. The cope is provided at the oposite end with an end member 15 which overlaps the end of the drag. The cope and drag may be provided on the longitudinal edges with interengaging flanges or ribs 16 which will hold the parts in proper alinement, but obviously will not prevent relative longitudinal movement. The parting line, designated 17, may be anywhere desired, and will be located according to the shape of the article to be cast. In a brakeshoe, it is preferably located between the face and back usually 35 nearer the back than the face. The drag is secured to any suitable support 18, while the cope is provided with any suitable means 19 for raising and handling same.

40 To enable the back strap, designated 20, to be supported in the mold prior to and during the casting operation, a large recess 21 is formed in the cope having an opening 22 which communicates with the interior of the mold, and through which the loop 23

45 of the back strap projects, the opening being preferably of such size that the loop fits snugly therein, so that the molten iron will not be able to flow up between the loop and the cope. The loop is provided with open-

50 ings 24 for keying the brakeshoe to a brake head, and these openings are made use of to secure the strap back in the mold in the following manner:—Hooks 25 of any suitable size and shape are provided which pass

55 through the recess 21 and engage in the openings 24 of the loop. These hooks may be supported in any suitable manner, such as by a taper pin 26 which passes through eyes 27 on the hooks. Preferably, though

60 not necessarily, the pin is tapered, so that it may be easily inserted and will draw the strap back tightly against the cope. In order to insure proper positioning of the back strap 20 and a uniform tension on the 65 hooks 25, the outer surface of the cope may

be provided with a slight depression 28, for the reception of the pin 26, so that the pin will always be located in exactly the same spot.

70 In carrying out the manufacture of brakeshoes according to this process, a back strap 20 is inserted in the cope, while the same is elevated above the drag. The hooks 25 are engaged in the openings of the strap loop, and the pin 26 pushed so as to draw equally 75 on the hooks 25 and support the back strap in the cope, and hold the same tightly against the surface of the cope so that molten iron will not enter between the strap and cope. This close engagement of the 80 back strap and cope is particularly important around the opening 22, as the strap acts as a seal for this opening and prevents the molten iron escaping therefrom into the recess 21. To guard against any leakage 85 of molten iron through the opening 22 due to a badly formed back strap, a small amount of sand, designated 29, may be thrown into the recess and the cope slightly agitated to cause the sand to work through 90 the openings 24 of the strap loop and entirely fill the lower part of the recess 21. The cope is lowered on the drag where it fits accurately by reason of the interengaging flanges 16 and the ends 13 and 15. The 95 molten metal is poured in through the runner 14 which is naturally located at the highest end of the mold. The metal runs down to the bottom of the mold and any air and gases trapped in the mold escape 100 through the vent 30 at the lower end. When the metal commences to solidify, it expands slightly, and if this expansion is greater than the expansion of the mold due to the transference of heat, the cope and drag will 105 be moved relatively to one another, so that they are not called upon to resist any force which would tend to burst them. In casting brakeshoes, the expansion of the metal on solidifying is very slight in the lateral and vertical directions, and in point of fact, owing to the position of the mold and the manner in which the metal accumulates therein, there is almost no expansion in these directions, but only in the longitudinal direction. Obviously, the only thing 110 that prevents the cope from moving in the vertical direction is its own weight, so that if there is any lateral expansion of the metal, it will still be soft enough to flow, 115 so that the expansion is transferred into either a vertical or a longitudinal direction or both. Owing to the position of the mold, a very perfect casting is obtained. The metal which first enters the mold is that 120 which forms the face of the shoe. If the metal stiffens on striking the cooler mold, the layer of molten metal above it operates to keep it soft and force it closely against the drag, so that a very smooth casting is 125 130

obtained. As the metal runs quietly down through the mold any bubbles of air or gas, which have been carried in with the metal, have ample time to separate from the metal 5 and are not imprisoned, as frequently occurs when the brakeshoe is poured vertically. Another advantage of this method is that the shoe may be said to cool from the face toward the back, whereas with vertical 10 pouring, the shoe cools from one end toward the other. The position in which the mold is arranged has numerous additional advantages; for example, any dross which may rise to the top of the metal will be 15 found at the back of the shoe in place of toward one end; so that the metal on the face of the shoe will be of even hardness throughout its length. There is in addition not nearly as much tendency for the metal 20 to force its way between the back strap and the cope or out through the opening 22, as would be the case if the mold was vertically disposed. A further advantage is that the cope may be lifted off the drag by an over- 25 head hoist, without disturbing the drag, and will not require anything but its own weight to hold it in position when on the drag.

In practice, it is obvious that more than 30 one mold will be used. The molds will be arranged in batteries, and the metal will be poured into them in succession. The number of molds in each battery will preferably be regulated, so that by the time the 35 last mold of the battery is opened and the casting removed, the first mold will be sufficiently cooled for the insertion of a new back strap and for the reception of a fresh charge of molten metal. In this 40 manner, the process of casting may be carried on continuously without any loss of time, and without having a large number of molds idle, for considerable periods of time.

It will also be seen that by carrying on this method of manufacture in a continuous 45 manner, the molds will, after the first few castings have been made, reach a temperature which they will maintain with very little variation. This is of considerable advantage, as it insures all castings being made 50 under exactly similar conditions.

While particular attention has been paid in the foregoing description to the casting of brake shoes, it must be understood that this is purely because brake shoes have been 55 selected as an example, and for the purpose of illustrating the method, so that the method is not limited to the casting of brake shoes, but may be applied to the casting of many other articles. 60

Having thus described my invention, what I claim is:

1. A method of making strap back brake-shoes, consisting in releasably maintaining the strap back tightly against the upper part 65 of a permanent mold by means applicable and removable from the exterior of the mold, and flowing molten metal under the strap.

2. A method of making strap back brake-shoes, consisting in holding a strap back tightly in the upper part of a mold by external means inserted through the mold, and flowing molten metal under the strap. 70

3. A method of making articles having 75 inserts of different material, which comprises holding the insert in an apertured mold by means inserted from the exterior of the mold through the aperture thereof, temporarily filling the aperture around the 80 holding means, and flowing molten metal into the mold.

In witness whereof I have hereunto set my hand.

MICHAEL J. WALSH.